

March 5, 1946.

W. L. KEENE

2,395,877

BIMETALLIC PRODUCTS AND MANUFACTURE THEREOF

Filed Jan. 22, 1942

Fig. 1.



Fig. 2.



Fig. 3.



Fig. 4.



Fig. 5.



Fig. 6.



Fig. 7.



INVENTOR

Walter L. Keene

by  
Sally and George  
his attorney

## UNITED STATES PATENT OFFICE

2,395,877

BIMETALLIC PRODUCTS AND  
MANUFACTURE THEREOFWalter L. Keene, Darment, Pa., assignee to  
Superior Steel Corporation, Pittsburgh, Pa., a  
corporation of Virginia

Application January 22, 1942, Serial No. 427,767

4 Claims. (Cl. 29—183)

This invention relates to bimetallic products and the manufacture thereof. It relates more particularly to the making and rolling of bimetallic billets or bars to form bimetallic material in sheet or strip form and, in turn, to the formation from such material of die-formed bimetallic shapes. Examples of such shapes are ammunition components such as bullet jacket cups and cartridge cases.

While in its broadest aspects the invention is applicable to a very wide variety of bimetallic products and the manufacture thereof, since at the present time it is of particular value and utility in connection with the manufacture of ammunition components it will be described as applied specifically to the manufacture of bullet jacket cups.

Bullet jackets are made by first forming preliminary cup-shaped blanks known as cups and then die-forming or drawing such cups into the finished jackets. Heretofore the cups have usually been made of a relatively soft corrosion resistant metal such as gilding metal or cupronickel. Such metal when used in bullet jackets has advantages which are well understood in the art. The soft metal avoids severe wear to the hard steel lands in the gun barrel and its corrosion resistance prevents rusting. However, such metals are relatively expensive. Also they are relatively low in structural strength, which in certain types of bullets is important. Consequently it is desirable to provide bullet jackets having the desirable properties of relatively soft corrosion resistant metal such as gilding metal or cupronickel and at the same time having the desirable properties of steel which here are relatively great structural strength and cheapness. This may be largely accomplished by making bullet jackets and, consequently, the intermediate cup-shaped blanks for formation into bullet jackets, out of a composite of steel and relatively soft corrosion resistant metal. Experiments looking toward the making of bimetallic material in sheet or strip form for formation into bullet jacket cups have been carried on for some time but until comparatively recently without thoroughly satisfactory results. Among the difficulties which have arisen has been the formation of bubbles and blisters between the layers of metal forming the composite bimetallic material. This has, I believe, been due largely to the absorption of hydrogen by the steel or other ferrous metal used as a component of the bimetallic material.

It is desirable to thoroughly pickle the ferrous metal component before forming the bimetallic billet; indeed it is desirable to severely pickle such component so as to roughen its surface to provide for most satisfactory union of the surfaces of the components of the bimetallic billet during hot rolling. In any event, the ferrous metal component must be thoroughly clean and this

is desirably accomplished by pickling. When the ferrous metal component consists of ordinary carbon steel it absorbs hydrogen during pickling and the hydrogen results in the formation of bubbles and blisters between the components of the bimetallic material during hot rolling. Baking has been resorted to in order to eliminate the absorbed or occluded hydrogen, but this is an undesirable, expensive and time-wasting step and the possibility exists that the very clean surfaces obtained by pickling will be less clean and free from oxides and other impurities after baking.

I have discovered that hydrogen absorption by the ferrous metal component of a bimetallic billet may be eliminated or at least reduced so that the effect of any absorbed hydrogen is negligible by employing a ferrous metal component having at least the surface portion or portions to which the other component or components of the billet is or are to be applied a carbon content not substantially exceeding .08%. When such a ferrous metal component is used baking is unnecessary and the other component or components of the billet may be applied thereto when the ferrous metal component is in its state immediately following pickling. In such state when the surface portion or portions of the ferrous metal component to which the other component or components of the billet is or are to be applied has or have a carbon content not substantially exceeding .08% such surface portion or portions is or are substantially free from absorbed hydrogen.

While it would be possible to employ a homogeneous ferrous metal component having throughout a carbon content not substantially exceeding .08% this would, at least in some instances, as, for example, in the manufacture of cartridge cases, be undesirable. In the manufacture of cartridge cases a relatively high yield point coupled with optimum ductility is desired and could not ordinarily be obtained or at least relied upon, when a homogeneous ferrous metal component having throughout a carbon content not substantially exceeding .08% is used. Moreover, such a homogeneous ferrous metal is costly and difficult to obtain. It is desirable that the ferrous metal component have as a whole a carbon content substantially exceeding .08% but that at least the surface portion or portions in question should have a carbon content not substantially exceeding .08%. While the component might be initially formed of homogeneous ferrous metal having a carbon content substantially exceeding .08% and have one or more surface portions decarburized, I have found it much more desirable and highly satisfactory in actual use to employ for formation of the ferrous metal component a rimming or capped steel whose surface has a carbon content not substantially ex-

ceeding .08% but which in the body portion thereof beneath the surface has a carbon content well above .08%. Such a steel not only desirably inhibits hydrogen absorption at the surface during pickling but is readily obtainable at reasonable cost and imparts to the component desirable physical properties which it would not have if the carbon content throughout the component were not substantially greater than .08%. While I am not certain as to the theory of action and make no representations with respect thereto, I believe that the fact that the outside layer of the rimming or capped steel component is relatively pure iron and low in carbon results in a much slower reaction between the metal and acid than is the case when ordinary carbon steel is used. I believe that as the reaction rate is slower the amount of hydrogen formed is less and consequently less hydrogen is absorbed.

When the ferrous metal component of a bimetallic billet is made out of metal of the character above described and such component is assembled with one or more other components to form the bimetallic billet and such billet is rolled into material in sheet or strip form and such material employed for the formation of cups the cups are found to be eminently satisfactory and the cost of production desirably low.

Other details, objects and advantages of the invention will become apparent as the following description of a present preferred embodiment thereof and a present preferred method of practicing the same proceeds.

In the accompanying drawing I have shown a present preferred embodiment of the invention and have illustrated a present preferred method of practicing the same, in which

Figure 1 is a cross-sectioned perspective view of a flanged ferrous metal component of a bimetallic billet;

Figure 2 is a similar view of a facing component;

Figure 3 is a similar view of the component shown in Figure 1 and two components such as shown in Figure 2 assembled but before the components are fastened together;

Figure 4 is a view similar to Figure 3 but showing the components of the billet fastened together;

Figure 5 is a view similar to Figures 1 to 4, inclusive, of hot rolled strip made from the billet shown in Figure 4;

Figure 6 is a similar view of cold rolled strip made from the hot rolled strip shown in Figure 5 and after shearing off the edges; and

Figure 7 is a central cross-sectional view through a bullet jacket cup formed from the cold rolled strip shown in Figure 6; the scale of Figure 7 being greater than that of the other figures.

Referring now more particularly to the drawing, there is shown in Figure 1 the ferrous metal component of a bimetallic billet, such component being designated by reference numeral 2. It comprises a body 3 and four flanges each designated 4. As shown in Figure 1, the flanges 4 are arranged in pairs, two flanges at the top of the component projecting generally upwardly in opposed relationship at the side edges of the component and two flanges at the bottom of the component projecting generally downwardly in opposed relationship at the side edges of the component. Thus channels are formed at the upper and lower faces of the component 2, viewing Figure 1, for the reception of the facing components, it being understood that the billet to

be formed is to have facing components top and bottom. A facing component is shown at 5 in Figure 2 and in Figure 3 the components 2 and 5 (there being two of the latter) are shown in assembled relationship but before being fastened together.

The component 2 is of ferrous metal, preferably steel. It may be formed by rolling, forging, milling or otherwise. It may be of any desired length.

10 As above mentioned, it is provided with channels top and bottom for receiving the facing components. Each such channel has a floor 6 and opposed side walls 7. The facing components lie against the respective floors 6 of the channels, 15 as shown in Figure 3. The metal of the component 2 at the surfaces thereof which form the floors 6 of the channels should have a carbon content not substantially exceeding .08%. The side walls 7 of the channels should preferably also have a carbon content not substantially exceeding .08%, although any bubbles or blisters forming at such side walls during hot rolling can ordinarily be squeezed out so that the gas will escape and not cause defects in the strip. It is 20 possible for the entire component 2 to be made of ferrous metal having a carbon content not substantially exceeding .08% and for certain uses such a component may be entirely satisfactory, although, as above pointed out, it is likely to be 25 expensive to obtain and its physical properties due to its low carbon content may not be as desired. I prefer to employ a rimming or capped steel whose carbon content at the surface is not substantially greater than .08% but whose carbon 30 content beneath the surface is substantially greater than .08%. I have found that such a steel is ideally suited to the formation of the ferrous metal component of a bimetallic billet as herein described. When a rimming or capped 35 steel is used the component 2 is preferably formed by rolling and the outside surface of the component will have a carbon content not substantially exceeding .08%, this including the surfaces 6 and the surfaces 7.

40 After the component 2 has been formed it is preferably thoroughly pickled to remove dirt, scale and oxides and provide, particularly at the surfaces 6 and 7, metallically clean faces for reception of the facing components. In many cases 45 it is desirable to carry the pickling step beyond the mere cleaning of the component and to severely pickle the component 2 sufficiently to roughen its surfaces. The purpose of this is primarily to roughen the surfaces 6 against which 50 the facing components lie to promote a strong union between the component 2 and the facing components 5 and insure against relative slippage therebetween during the hot rolling.

I prefer to employ a 5% solution of sulphuric 55 acid at a temperature of 160 to 180° F. for the pickling step. When it is desired to roughen the surface of the component 2 such component will be left in the pickling tank for a time which may approach or possibly slightly exceed two 60 hours. In such time when a steel of the type above mentioned is employed the surfaces will of course be thoroughly cleaned and will also be desirably roughened. When the component 2 is subjected to a severe pickle such as just mentioned, if the carbon content of the metal thereof 65 at the surface is substantially greater than .08% there will be undesirable hydrogen absorption or occlusion which when the bimetallic billet is formed and rolled will, as above stated, result 70 in the formation of bubbles and blisters between 75 the surfaces 6 and 7.

the layers of metal. Such bubbles and blisters destroy the bond between the components and render at least portions and possibly all of the rolled bimetallic material unsatisfactory for use. I have found that when the carbon content of at least the faces 6 of the component 2 is not substantially greater than .08% the component will withstand a severe pickle without absorbing enough hydrogen to result in the formation of blisters or bubbles. When, for example, a rimming or capped steel whose outer surface has a carbon content not substantially exceeding .08% is used for formation of the component 2 such component can be immersed for two hours in 5% sulphuric acid at a temperature of 160 to 180° F. without undesirable hydrogen absorption. This is as severe a pickle as is likely to be desired at any time.

When the component is removed from the pickling bath it is preferably washed off with water and then dipped in sodium carbonate which tends to neutralize any remaining acid. This may be followed by a soak in hot water which aids in rapid drying of the component.

The components 5 are ordinarily of non-ferrous metal such as copper, brass, gilding metal, cupronickel or other relatively soft corrosion resistant alloy. For example, I prefer to use a gilding metal which has a copper content of in the neighborhood of 90% and a zinc content of in the neighborhood of 10%. Cupro-nickel having a copper content of in the neighborhood of 80% and a nickel content of in the neighborhood of 20% is also entirely satisfactory.

The facing components as well as the component 2 are thoroughly cleaned and the facing components may likewise be severely pickled to roughen them. They are assembled as shown in Figure 3 whereafter the flanges 4 are deformed inwardly to firmly hold the components 5 in place and form a bimetallic billet ready for rolling as shown in Figure 4. The billet may take various forms, that shown in Figure 4 being merely an example. For rolling sheets a bimetallic sheet bar may be similarly or otherwise formed. Such billet or bar when hot rolled forms strip or sheets as shown in Figure 5 in which the metal of the component 2 is faced at its central portion with the metal of the components 5. Herein the word "billet" is used generically to include billets and bars and the word "strip" is used generically to include any metal in strip or sheet form.

During the hot rolling the components or layers of the bimetallic material are disposed in face-to-face contact and have their contacting faces united to each other substantially throughout their area of contact. The union is believed to be in the nature of a mechanical bond or weld, apparently being accomplished by the combination of heat and pressure.

The strip is preferably cold rolled and either before or after the cold rolling step the edges which consist entirely of the metal of the component 2 are sheared off, forming cold rolled strip as shown in Figure 6. Such strip is used for formation of cups as shown in Figure 7. The particular cup shown in Figure 7 is a bullet jacket cup adapted for further die-forming operations to form a finished bullet jacket. Similar cups may be formed for formation into cartridge cases, shells or other ammunition components. Similar or other generally cup-shaped blanks may likewise be formed for a wide variety of other purposes or the metal in sheet or strip form may be otherwise employed.

The product formed in accordance with my invention is of high quality and free from bubbles or blisters between the layers of metal and may be made at a cost comparing favorably with the cost of making similar products entirely out of non-ferrous metal. Although a severe pickle of the ferrous metal component of the billet may be and preferably is employed the amount of hydrogen absorption if any is negligible from the standpoint of formation of bubbles and blisters during hot rolling. Baking to remove absorbed or occluded hydrogen is unnecessary. The product, in addition to being of high and uniform quality, possesses adequate mechanical strength and desirable physical properties.

While I have shown and described a present preferred embodiment of the invention and a present preferred method of practicing the same it is to be distinctly understood that the invention is not limited thereto but may be otherwise variously embodied and practiced within the scope of the following claims.

I claim:

1. A method of making a bimetallic billet comprising providing a component of rimming or capped steel having a surface having a carbon content not substantially exceeding .08%, severely pickling said component so as to substantially roughen its surface, applying to said component in its state immediately following pickling and in contact with said surface a component of gilding metal and fastening said components firmly together.

2. A bimetallic billet for rolling comprising a pickled steel component having a surface having a carbon content not substantially exceeding .08% and in its state immediately following pickling being by reason of the aforementioned carbon content substantially free from absorbed hydrogen and a second preformed metal component lying against said surface, said components being firmly held together ready for rolling, said freedom of said first mentioned component from absorbed hydrogen providing for substantial freedom from bubbles and blisters between said components when the billet is hot rolled.

3. A bimetallic strip comprising a pickled steel component having a surface having a carbon content not substantially exceeding .08% and in its state immediately following pickling being by reason of the aforementioned carbon content substantially free from absorbed hydrogen and a second metal component lying against said surface, said components being welded together substantially throughout their area of contact, said freedom of said first mentioned component from absorbed hydrogen providing for substantial freedom from bubbles and blisters between said components during rolling of the strip.

4. A bimetallic billet for rolling comprising a component of pickled rimming or capped steel having a surface having a carbon content not substantially exceeding .08% and in its state immediately following pickling being by reason of the aforementioned carbon content substantially free from absorbed hydrogen and a second metal component lying against said surface, said components being firmly held together ready for rolling, said freedom of said first mentioned component from absorbed hydrogen providing for substantial freedom from bubbles and blisters between said components when the billet is hot rolled.